

# UNITED STATES PATENT OFFICE.

LOUIS CROSSMAN, OF NEW YORK, N. Y.

## UNDERCOATING COMPOSITION.

1,425,510.

Specification of Letters Patent. Patented Aug. 15, 1922.

No Drawing.

Application filed February 8, 1922. Serial No. 535,065.

To all whom it may concern:

Be it known that I, Louis CROSSMAN, a citizen of the United States, residing at New York, in the county of New York and State of New York, have invented certain new and useful Improvements in Under-coating Compositions, of which the following is a specification.

This invention relates to an under-coating composition for paint, enamel, and varnish, the object of the invention being to provide an improved under-coating composition, the use of which will save the use of several coats of paint in ornamenting or protecting surfaces.

As is well known painted surfaces require usually a number of coats of paint in order to thoroughly and efficiently cover the same, and where these surfaces are particularly porous or green a comparatively large number of coats of paint have to be used before the final coat can be effectively applied, and the use of so many coats of paint is expensive not only because of the time required to apply the numerous coats but also because of the cost of the materials which make up the paint. I have found however that by the use of the present composition, one coat thereof not only acts as a filler and covers the pores of the surface to be treated, but that this one coat gives a glazed surface which does not soak into the wood or other surface which it covers, and takes the place of two or three more coats of paint, and as it is comparatively inexpensive to manufacture, it follows that not only is the labor of applying the extra coats of paint eliminated but also the cost of such coats of paint.

This improved composition comprises essentially celluloid, acetone to dissolve it, alcohol, and preferably a small quantity of shellac. In practice I prefer also to use benzole as this thins down the acetone, and as this is cheaper, less acetone has to be used. I also prefer to use a small quantity of acetic acid as this offsets the odor of the acetone, and I also prefer to use a small quantity of amyl-acetate which tends to prevent the composition after it is applied from turning white. Therefore in practice in its preferred form this under-coating composition, approximately per gallon thereof comprises substantially about  $\frac{8}{16}$  gallon of acetone,  $\frac{1}{16}$  gallon wood alcohol,  $\frac{1}{16}$  gallon benzole, 2 oz. of celluloid, 1 oz.

of shellac,  $\frac{1}{2}$  oz. of acetic acid, and  $\frac{1}{2}$  oz. of amyl-acetate. The acetone, with the assistance of the wood alcohol dissolves the celluloid. The benzole thins down the acetone, the shellac serving to somewhat harden the composition.

The cost per gallon is about \$1.05 at the present time while the cost of paint varies according to the quality thereof from approximately \$3.00 up, and since one coat of this composition applied to a surface will act to permit the final coat of paint to be applied, it will be immediately apparent that there will not only be a great saving in the cost of the time and labor of applying several coats of paint, but also in the cost of the paint required to do the work.

I have found in practice also that this composition may be effectively used to cover wall paper, and thereby enable it to be readily washed.

As a practical painter and decorator I have been using this material for some time past with very great success with the result that I am able to do and efficient and satisfactory decorating job in a day or two which would ordinarily take a week, since the under-coating quickly dries thus enabling the last coat to be very promptly applied.

I have also found that wood covered and protected by this under-coating and then painted or enamelled, can be struck with a hammer without the enamel cracking or chipping off, which is not possible with wood covered with a primary and several other coats of paint. Scraps of celluloid or old films may be used effectively.

Thus by the use of a single coating of this composition, the necessity of a primary coat and several intermediate coats of paint before the application of the final coat is entirely eliminated.

If desired the under-coating may be colored by the use of any suitable coloring material or pigment. It will be understood that I do not limit myself to the exact proportions of the ingredients as these may be somewhat varied, nor necessarily to the use of all of the ingredients hereinbefore referred to as these likewise may be somewhat varied in accordance with the surface to be treated.

I claim as my invention:

1. An under-coating composition for surfaces comprising acetone, alcohol, and celluloid, the acetone being in greater proportion

than the alcohol, the wood alcohol being in less proportion than the acetone.

2. An under-coating composition for surfaces comprising wood alcohol, acetone, and celluloid.

3. An undercoating composition for surfaces comprising alcohol, acetone, celluloid, and shellac.

4. An under-coating composition for surfaces comprising alcohol, acetone, celluloid, shellac, and amyl-acetate.

5. An under-coating composition for surfaces comprising alcohol, acetone, celluloid, shellac, amyl-acetate, and acetic acid.

10 6. An under-coating composition for surfaces comprising acetone, wood alcohol, benzole, and celluloid.

7. An under-coating composition for surfaces comprising acetone, wood alcohol, benzole, celluloid, and shellac.

20 8. An under-coating composition for surfaces comprising acetone, wood alcohol, benzole, celluloid, shellac, and amyl-acetate.

9. An under-coating composition for surfaces comprising acetone, wood alcohol, 25 benzole, celluloid, shellac, amyl-acetate, and acetic acid.

10. An under-coating composition for surfaces comprising approximately for each gallon,  $\frac{8}{16}$  gallon acetone,  $\frac{15}{16}$  gallon wood 30 alcohol,  $\frac{1}{16}$  gallon benzole, and 2 ounces of celluloid.

11. An under-coating composition for surfaces comprising approximately for each gallon,  $\frac{8}{16}$  gallon acetone,  $\frac{15}{16}$  gallon wood 35 alcohol,  $\frac{1}{16}$  gallon benzole, 2 ounces celluloid, 1 ounce shellac, and  $\frac{1}{2}$  ounce amyl-acetate.

12. An under-coating composition for surfaces comprising approximately for each gallon,  $\frac{8}{16}$  gallon acetone,  $\frac{15}{16}$  gallon wood 40 alcohol,  $\frac{1}{16}$  gallon benzole, 2 ounces celluloid, 1 ounce shellac,  $\frac{1}{2}$  ounce amyl-acetate, and  $\frac{1}{2}$  ounce acetic acid.

Signed at 1822 Park Row Building, New York, N. Y., this 7th day of February, 1922. 45

LOUIS CROSSMAN.